# EUROPEAN PATENT SPECIFICATION

(11) **EP 0 941 209 B1**
(45) Date of publication and mention of the grant of the patent: **20.08.2003**
(21) Application number: 98940444.7
(22) Date of filing: 01.09.1998
(51) Int. Cl.: B68G 1/00, A47G 9/00, D01F 2/02, D04H 1/00, D04H 1/42, D04H 1/02

(54) **FILLING COMPRISING A POLYESTER FIBRE**
POLYESTERFASER ENTHALDENDES POLSTERMATERIAL
MATIERE DE REMBOURRAGE CONTENANT DE LA FIBRE DE POLYESTER

(30) Priority: 26.09.1997 GB 9720436
(43) Date of publication of application: 15.09.1999
(73) Proprietor: Trendsetter Home Furnishings Limited, Oldham OL8 4JY (GB)
(72) Inventor: BLACK, Robert, Paul, Cheshire WA6 9EZ (GB)
(74) Representative: W.P. Thompson & Co.
(86) International application number: GB9802619
(87) International publication number: WO99016705

(56) References cited:
- EP-A- 0 474 300
- WO-A-93/06806
- WO-A-96/09546
- GB-A- 1 486 639
- US-A- 5 311 389
- PATENT ABSTRACTS OF JAPAN vol. 098, no. 008, 30 June 1998 & JP 10 072771 A (ASAHI CHEM IND CO LTD), 17 March 1998

## Description

The present invention relates to a padding, stuffing or filling material comprising a polyester fibre. Such a material is known from the document EP-A-0474300 which represents the preamble of claim 1. More particularly it relates to an improved polyester fibre containing filling for use where thermal properties and/or breathability are important, such as in the soft furnishings industry, where it may be used as a filling for bedding, for example duvets, pillows, mattress protectors and sleeping bags or in the clothing industry where it may be used as a filling for coats, anoraks, and the like, particularly ski and winter wear.

Polyester fibre, usually polyethyleneterephthalate, is an inexpensive alternative to down or feathers. However it lacks breathability. In an attempt to improve the characteristics of a filling comprising polyester fibre, the polyester fibre has been blended with natural materials such as, for example, cotton, silk, down and feather.

Considerable effort has been made in the industry to provide an improved synthetic filling and in particular one with improved breathability.

It is an aim of the present invention to provide a synthetic fibrefill with improved breathability but which retains at least some of the desirable properties of polyester fibrefill.

It has unexpectedly been found that cellulosic fibres obtained by an organic solvent spinning process, according to claim 1, and in particular one in which the organic solvent is N-methyl morpholine oxide (NMMO) e.g. lyocell, when blended (in contrast to woven) with a polyester filling fibre such as, for example, polyethyleneterephthalate gives rise to a product with improved characteristics including improved breathability compared to a polyester filling fibre alone. The finding was unexpected given that lyocell fibres are traditionally flat and would not have been expected to be a good filling fibre. Lyocell is a cellulosic fibre made by direct dissolution of wood pulp in an organic solvent and has to date been used primarily in the development of technical textiles, namely woven fabrics comprising interlaced warp and weft threads.

It is another aim of the present invention to provide a synthetic fibrefill with improved thermal performance.

It has unexpectedly been found that cellulosic fibre e.g. lyocell, when blended with a polyester filling fibre, such as, for example, polyethyleneterephthalate gives rise to a product with improved thermal characteristic compared to the component fibres alone.

According to the present invention there is provided a non-woven blend comprising or consisting of a polyester filling fibre and a cellulosic fibre obtained by an organic spinning process.

Preferably the cellulosic fibre is lyocell.

Preferably the polyester filling fibre is polyethyleneterephthalate fibre.

Preferably the blend comprises, by weight, no more than 80%, more preferably still 60%, of the cellulosic fibre, for example, lyocell.

More preferably the cellulosic fibre, for example, lyocell is present in an amount of from 10 - 60% by weight and ranges therebetween, more preferably still 20- 60% and more preferably still from 25- 60% of the blend.

Preferably the polyester filling fibre comprises mono fibres which are crimped or conjugate fibres. By conjugate fibres is meant fibres comprising two different fibre-forming polymeric units arranged side by side so that on heat treatment the fibre becomes spirally crimped.

Preferably the cellulosic or lyocell fibre is a saw-toothed crimp fibre.

More preferably the cellulosic or lyocell fibres and polyester filling fibres are formed into a fibre ball. To form a fibre ball it is preferred to use a lyocell cellulosic fibre blended with a conjugate polyester preferably of polyethyleneterephthalate.

Alternatively a lyocell cellulosic fibre and either a conjugate polyester or a regular saw tooth crimp polyester fibre are blended, carded and layered into a wadding. For the avoidance of doubt a wadding is neither a woven product nor a fabric.

Preferably the wadding is more than 3 mm thick and more preferably more than 5 mm thick. It is a loose open material in contrast to compressed materials such as for example felts.

According to a further aspect of the present invention there is provided a bedding article comprising as a filling a non-woven blend of the invention.

According to a further aspect of the present invention there is provided an article of clothing comprising as a filling a non-woven blend of the invention.

The bedding article may be, for example, a duvet, pillow, quilt, sleeping bag, cushion or other similar article.

The clothing article may be, for example, a jacket, coat, or anorak.

The non-woven blend has characteristics which make it more desirable than a polyester filling, for example, polyethyleneterephthalate alone:
1) it has a more down like feel;
2) weight for weight it is warmer than polyethyleneterephthalate; and
3) It is breathable, i.e. moisture absorbent;

Fibreballs of the non-woven blend also show improved breathability and thermal properties.

The blending of fibres, and the production of fibre balls are well known processes to the man skilled in the art and are not therefore described herein.

The invention will be further described, by way of example only, with reference to the tabulated test data shown in tables 1 and 2 below:
Table 1 shows the products under test; and
Tables 2 and 3 show the properties of the products under test.

It should be noted with reference to table 1 that pure lyocell has a fill weight of 49.3 gm/m²/tog, which is similar to the figure of 49 gm/m²/tog for pure polyester. The blend however gives a figure of 39 gm/m²/tog ie a synergistic and non obvious effect is achieved with a mixture.

**TABLE 1**

| | Duvet Weight | U.K. Tog Test | Fill wgt gm/m²/tog |
|---|---|---|---|
| Cellulosic/ Polyester Carded Blend | 2060g | 13.5 | 37 |
| Goose down | 1790g | 13.5 | 18 |
| Hollow Polyester fibre Carded | 2488g | 13.5 | 49 |

It will be noted from test results shown in tables 2 and 3 that the non-woven blend of the invention is significantly better than pure polyester (the current synthetic filling of choice) when it comes to its thermal insulation properties, its water vapour permeability index, its ratio of thermal insulation to weight, its thermal physiological comfort, its water vapour take up and its buffering capacity moisture transport and uptake properties and only insignificantly worse in its effective water vapour resistance. In other words, the non-woven blend confers a higher degree of thermal insulation and possesses better moisture transport properties under stationary conditions combined with better moisture absorption than a pure polyester material.

## Claims

1. A padding, stuffing or filling material comprising a non-woven blend including a polyester filling fibre **characterised in that** the blend includes a cellulosic fibre obtained by an organic spinning process.

2. A padding, stuffing or filling material according to claim 1 wherein the cellulosic fibre is Lyocell.

3. A padding, stuffing or filling material according to claim 1 or claim 2 wherein the polyester filling fibre is polyethyleneterephthalate fibre.

4. A padding, stuffing or filling material according to any one of the preceding claims, comprising, by weight, no more than 80% of the cellulosic fibre.

5. A padding, stuffing or filling material according to any one of the preceding claims, wherein the cellulosic fibre is present in an amount, by weight, of from 10-60% of the blend.

6. A padding, stuffing or filling material according to any one of the preceding claims wherein the cellulosic fibre is present in an amount, by weight, of from 20-60% of the blend.

7. A padding, stuffing or filling material according to any one of the preceding claims wherein the cellulosic fibre is present in an amount, by weight, of from 25-60% of the blend.

8. A padding, stuffing or filling material according to any one of the preceding claims wherein the polyester filling fibre comprises monofibres which are crimped or conjugate fibres.

9. A padding, stuffing or filling material according to any one of the preceding claims wherein the polyester filling fibre comprises conjugate fibre.

10. A padding, stuffing or filling material according to any one of the preceding claims wherein the cellulosic fibre is a saw-toothed crimp fibre.

11. A padding, stuffing or filling material according to any one of the preceding claims wherein the non-woven blend is in the form of fibreballs.

12. A padding, stuffing or filling material according to any one of the preceding claims wherein the non-woven blend is carded and layered in the form of a wadding.

13. An insulating material comprising the padding, stuffing or filling material according to any one of the preceding claims.

14. A bedding article comprising a padding, stuffing or filling material as claimed in any one of the preceding claims.

15. A bedding article as claimed in claim 13 selected from the group consisting of a duvet, pillow, mattress, mattress protector, sleeping bag, topper, quilt, enhancer, comforter and a bed.

16. An article of clothing comprising a padding, stuffing or filling material as claimed in any one of claims 1 to 12.

17. An article of clothing as claimed in claim 15 selected from the group consisting of a coat, jacket, anorak, and ski or winter wear.

## Patentansprüche

1. Wattier-, Polster- oder Füllmaterial, umfassend, eine Non-Woven-Mischung, einschließlich einer Polyesterfüllfaser, **dadurch gekennzeichnet, dass** die Mischung eine durch ein organisches Spinnverfahren erhaltene Cellulosefaser einschließt.

2. Wattier-, Polster- oder Füllmaterial nach Anspruch 1, worin die Cellulosefaser Lyocell ist.

3. Wattier-, Polster- oder Füllmaterial nach Anspruch 1 oder 2, worin die Polyesterfüllfaser Polyethylenterephthalat-Faser ist.

4. Wattier-, Polster- oder Füllmaterial nach einem der vorangehenden Ansprüche, umfassend nicht mehr als 80 Gew.-% der Cellulosefaser.

5. Wattier-, Polster- oder Füllmaterial nach einem der vorangehenden Ansprüche, worin die Cellulosefaser in einer Menge von 10 - 60 Gew.-% der Mischung vorliegt.

6. Wattier-, Polster- oder Füllmaterial nach einem der vorangehenden Ansprüche, worin die Cellulosefaser in einer Menge von 20-60 Gew.-% der Mischung vorliegt.

7. Wattier-, Polster- oder Füllmaterial nach einem der vorangehenden Ansprüche, worin die Cellulosefaser in einer Menge von 25 - 60 Gew.-% der Mischung vorliegt.

8. Wattier-, Polster- oder Füllmaterial nach einem der vorangehenden Ansprüche, worin die Polyesterfüllfaser Einzelfasern umfasst, die Kräusel- oder Bikomponentenfasern sind.

9. Wattier-, Polster- oder Füllmaterial nach einem der vorangehenden Ansprüche, worin die Polyesterfüllfaser eine Bikomponentenfaser umfasst.

10. Wattier-, Polster- oder Füllmaterial nach einem der vorangehenden Ansprüche, worin die Cellulosefaser eine Sägezahn-Kräuselfaser ist.

11. Wattier-, Polster- oder Füllmaterial nach einem der vorangehenden Ansprüche, worin die Non-Woven-Mischung in der Form von Faserkügelchen vorliegt.

12. Wattier-, Polster- oder Füllmaterial nach einem der vorangehenden Ansprüche, worin die Non-Woven-Mischung in der Form einer Wattierung kardiert und geschichtet ist.

13. Isoliermaterial, umfassend das Wattierungs-, Polster- oder Füllmaterial nach einem der vorangehenden Ansprüche.

14. Bettzeug-Artikel, umfassend ein Wattier-, Polster- oder Füllmaterial nach einem der vorangehenden Ansprüche.

15. Bettzeug-Artikel nach Anspruch 13, ausgewählt aus der Gruppe, bestehend aus einem Deckbett, einem Kissen, einer Matratze, einem Matratzenschützer, einem Schlafsack, einer Auflage, einer Quiltdecke, einem Enhancer, einer Steppdecke und einem Bett.

16. Kleidungsartikel, umfassend ein Wattier-, Polster- oder Füllmaterial nach einem der Ansprüche 1 bis 12.

17. Kleidungsartikel nach Anspruch 15, ausgewählt aus der Gruppe, bestehend aus einem Mantel, einer Jacke, einem Anorak und Ski- und Winterkleidung.

## Revendications

1. Matériau de matelassage, de rembourrage ou d'emplissage comprenant un mélange non tissé comportant une fibre d'emplissage en polyester, **caractérisé en ce que** le mélange comporte une fibre cellulosique obtenue par un procédé de filage organique.

2. Matériau de matelassage, de rembourrage ou d'emplissage selon la revendication 1, dans lequel la fibre cellulosique est le Lyocell.

3. Matériau de matelassage, de rembourrage ou d'emplissage selon la revendication 1 ou la revendication 2, dans lequel la fibre d'emplissage en polyester est une fibre de polyéthylènetéréphtalate.

4. Matériau de matelassage, de rembourrage ou d'emplissage selon l'une quelconque des revendications précédentes, comprenant, en poids, au plus 80% de fibre cellulosique.

5. Matériau de matelassage, de rembourrage ou d'emplissage selon l'une quelconque des revendications précédentes, dans lequel la fibre cellulosique est présente en une quantité, en poids, allant de 10 à 60% du mélange.

6. Matériau de matelassage, de rembourrage ou d'emplissage selon l'une quelconque des revendications précédentes, dans lequel la fibre cellulosique est présente en une quantité, en poids, allant de 20 à 60% du mélange.

7. Matériau de matelassage, de rembourrage ou d'emplissage selon l'une quelconque des revendications précédentes, dans lequel la fibre cellulosique est présente en une quantité, en poids, allant de 25 à 60% du mélange.

8. Matériau de matelassage, de rembourrage ou d'emplissage selon l'une quelconque des revendications précédentes, dans lequel la fibre d'emplissage en polyester comprend des monofibres qui sont des fibres crêpées ou conjuguées.

9. Matériau de matelassage, de rembourrage ou d'emplissage selon l'une quelconque des revendications précédentes, dans lequel la fibre d'emplissage en polyester comprend des fibres conjuguées.

10. Matériau de matelassage, de rembourrage ou d'emplissage selon l'une quelconque des revendications précédentes, dans lequel la fibre cellulosique est une fibre crêpée en dents de scie.

11. Matériau de matelassage, de rembourrage ou d'emplissage selon l'une quelconque des revendications précédentes, dans lequel le mélange non tissé est sous forme de balles de fibres.

12. Matériau de matelassage, de rembourrage ou d'emplissage selon l'une quelconque des revendications précédentes, dans lequel le mélange non tissé est cardé et mis en couches sous forme d'un ouatage.

13. Matériau isolant comprenant le matériau de matelassage, de rembourrage ou d'emplissage selon l'une quelconque des revendications précédentes.

14. Article de literie, comprenant un matériau de matelassage, de rembourrage ou d'emplissage selon l'une quelconque des revendications précédentes.

15. Article de literie selon la revendication 13, choisi parmi le groupe constitué par un duvet, un oreiller, un matelas, une alèse, un sac de couchage, un sur-matelas, une couverture piquée, un édredon, une couette et un lit.

16. Article vestimentaire, comprenant un matériau de matelassage, de rembourrage ou d'emplissage selon l'une quelconque des revendications 1 à 12.

17. Article vestimentaire selon la revendication 15, choisi parmi le groupe constitué par un manteau, une veste, un anorak, et des vêtements de ski ou d'hiver.
